# EUROPEAN PATENT SPECIFICATION

(11) **EP 1 507 919 B1**
(45) Date of publication and mention of the grant of the patent: **26.03.2008**
(21) Application number: 02736309.2
(22) Date of filing: 21.05.2002
(51) Int. Cl.: D06M 16/00, C12N 11/08

(54) **TREATMENT OF ANIMAL HAIR FIBERS WITH MODIFIED PROTEASES**
BEHANDLUNG VON TIERISCHEN HAARFASERN MIT MODIFIZIERTEN PROTEASEN
TRAITEMENT DE FIBRES D'ORIGINE ANIMALE AVEC DES PROTEASES MODIFIEES

(43) Date of publication of application: 23.02.2005
(73) Proprietor: Universidade do Minho, 4700-320 Braga (PT)
(72) Inventor: CAVACO PAULO, Artur, 4715-191 Braga (PT); DOS SANTOS MARINHO DA SILVA, Carla, Joana, P-4710 Braga (PT)
(74) Representative: Silva Carvalho, Luis Manuel
(86) International application number: PCT/PT2002/000008
(87) International publication number: WO 2003/097927

(56) References cited:
- WO-A-00/50686
- WO-A-99/60200
- US-A- 4 970 156
- DATABASE WPI Section Ch, Week 199509 Derwent Publications Ltd., London, GB; Class A35, AN 1995-064089 XP002229518 & JP 06 341067 A (OSAKA PREFECTURE), 13 December 1994 (1994-12-13)

## Description

### Field of the invention

The cuticle layer of animal hair fibres presents a scaly structure when observed by microscopy. The felting or shrinkage of these fabrics is due to the overlapping of these scales that surround the cortex (inner part of the fibre), in wet processes with high mechanical agitation. The removal of the cuticle layer makes it possible to eliminate the tendency of the protein fibres of animal origin to shrink. One possibility of anti-felt treatment would be the application of proteolytic treatments for the removal of the cuticle layer. This kind of treatment has been extensively studied since the beginning of the 20^{th} century, but without great achievements.

The reasons for this are primarily due to the following factors:
- The hair fibres of animal origin have a very variable composition, which depends on origin, race, climate and animal feeding. This diversity of animal fibres induces several susceptibilities to the proteolytic treatments.
- More aggressive treatments to induce a uniform anti-felting behaviour to all the fibres consequently cause unacceptable loss of strength.
- Recent studies indicate that the lack of reproducibility of the proteolytic treatments and the degradations caused by such treatments are due to the diffusion of the enzymes inside the animal fibres.

### Background of the invention

The most commonly used method to confer dimensional stability to articles made from animal hair fibres is the INS/CSIRO Chlorine/Hercosett, which comprises a strong acid chlorine treatment, followed by the application of a polymer resin. This process results in an increased degree of shrinking resistance, but has a number of drawbacks: poor feel, limited durability, difficulties in dyeing and, more importantly today, it generates environmentally damaging waste.

Several authors have suggested methods to reduce the shrinkage of animal fibres, such as wool for instance, which do not result in the release of substances that are harmful to the environment. Among such processes, there are the enzymatic ones, as well as benign chemical processes such as low-temperature plasma treatments. Plasma treatment is a dry process, which involves treating wool fibre material with electric gas discharges (so-called plasma). At present, there are serious obstacles such as costs, compatibility and capacity, to large-scale commercialisation of a plasma treatment process.

Several enzymatic methods have been used for wool treatments. The patent JP 6341067 describes the use of water-soluble immobilized proteases for the treatment of several textile materials, where the enzyme can be recovered and reused. This patent however does not describe the use of activating agents and therefore free enzymes could be also present in solution. The patent JP-A 51099196 describes a process to treat wool fabrics with alkaline proteases. The patent JP-A 3213574 describes a method for the treatment of wool with transglutaminase or a solution having this enzyme. The patents US 6051033 describe a method of wool or wool fibres treatment with a proteolytic enzyme and transglutaminase. WO 98/27264 describes a method to reduce the shrinking of wool that consists of bringing the fibre samples into contact with a solution of peroxidase or oxidase under the adequate conditions for the enzymatic reaction with wool. The patent US 6099588 relates a method to improve shrink resistance that may result in improvements in feel, appearance and felting, among others, by the application of proteolytic enzymes in an aqueous solution, after treatment with an alkaline solution containing alcohol. The patent US 5.529.928 refers to a process for obtaining wool with anti-felt finishing, a soft feel and with shrink resistance using an initial chemical oxidation followed by a treatment with protease and warming. The patent EP 134267 uses a similar process, treating the fibre with proteolytic enzymes in the presence of salt, after the initial oxidative treatment. The patent EP 3.58386 describes a method of wool treatment that consists of a proteolytic treatment and one of, or both, an oxidative treatment (such as NaOCl) and treatment with polymer.

The necessity of establishing environmentally friendly (Eco-friendly) methods with better performances than the industrial processes currently used, creates a need for new processes that give a good shrink resistance, softness, appearance and anti-pilling behaviour. Therefore, a new methodology of enzymatic treatment of animal hair fibres is presented here.

### Summary of the invention

This invention relates to a new anti-felting method of treating animal hair fibres characterized by the contact of the animal hair fibres with a solution of proteases that were chemically modified by glutaraldehyde and/or γ-aminopropyltriethoxysilane to increase its molecular weight in order to reduce their diffusion inside the fibre. The cuticle will be the only accessible part to the proteolytic attack, which allows for the improvement of one or more wool properties, including their felting and shrinking, without damaging the fibre's interior.

The methodologies used to increase the molecular weight of the enzymes are based on the utilization of a soluble polymer with hydroxyl groups activated with γ-aminopropyltriethoxysilane and/or glutaraldehyde. The glutaraldehyde may subsequently bind to another polymer chain, forming a polymeric net, or to an available protein NH₂ group.

### Detailed description of the invention

The method consists in the treatment of the protein material with a solution of modified proteolytic enzymes. Commercially available proteases from Sigma (*Subtilisin* kind) were used.

The immobilisation was performed on a soluble polymer, polyvinyl alcohol (Sigma), of average molecular weight 70000-100000, using glutaraldehyde (Aldrich), γ-aminopropiltrietoxisylane, and/or Borax (Sigma) and polyethylenglycol (Sigma) of 10000 of average molecular weight.

The polymer at 6% (w/v) solution in distilled water was dissolved with warming and stirring, activated, and then was added to a 2% (v/v) glutaraldehyde solution. This solution was kept under stirring at room temperature, for 2 hours. After this time, the solution was dialysed in 0.1 M pH 5.0 acetate buffer for 24 hours and then in 0.05 M pH 3.95 acetate buffer for 20 hours.

The enzymatic preparation in the desired concentration was added to the resulting solution, together with PEG (1.25%) and Borax (0.05 µg/mL) in 0.1 M pH 5.0 acetate buffer, and kept under stirring for 8 hours at room temperature. This solution was kept at 4°C until use. The immobilisation procedure did not cause any significant loss in activity.

### Example 1:

### Treatment of pure wool fabric with proteases:

Samples of pure merino wool fabric (like animal hair fibre) with about 12 cm x 12 cm (of about 3 grams, each), were placed in a recipient containing a solution of proteases being chemically modified or not, in a relation of 1/20 (w/v). The treatment was performed at 37°C, for periods of time ranging from 4 to 48 hours. The samples were removed from the solution, washed and air-dried. They were then subjected to tests to evaluate possible damage caused during the treatment.

To evaluate the quality of the fabric and the degree of damage caused in the wool treatment process, a qualitative test based on Garner (Garner W., Textile Laboratory Manual, vol. 5 - Fibres, 3rd Edition, 1967) was used. It was verified that the modified proteases did not induce fibre degradation when compared with free proteases. The control treatment itself (10 mM pH 7.5 acetate buffer) presents a level of degradation higher than that presented by the fibres treated with modified enzymes.

The tendency of the fabrics to shrink was verified by washing the fabrics (11 x 6 cm) three times in distilled water containing 50 µL of a wetting agent for 60 minutes, at 50°C and 20 rpm, and the shrinkage was measured by the variation of the specimen dimensions. It was verified that only the enzymatically treated fabrics did not induce a significant shrinkage.

A panel of 5 experts evaluated the feel and appearance of the wool fabric, verifying an increase in the properties of the protease treated fabrics compared to the control fabric.

### Example 2:

### Treatment of pure wool yarns with proteases:

Similar studies were conducted in yarns of merino wool using the following parameters: samples of pure wool yarn were placed in a recipient containing a solution of proteases being chemically modified or not, in a bath ratio of 1/20 (w/v). The treatment was conducted at 37°C, for periods of time ranging from 4 to 48 hours. The samples were removed from the solution, washed and air-dried. They were then subjected to test to evaluate possible damage caused during treatment.

To evaluate the yarn quality and the degree of damage caused in the treatment process of this fibre, a qualitative test based on Garner (Garner W., Textile Laboratory Manual, vol. 5 - Fibres, 3rd Edition, 1967) was used. It was verified that the modified protease treatment does not induce degradation when compared with free protease treatment. The control treatment (10 mM pH 7.5 acetate buffer) presented a level of degradation higher than that presented by the fibres treated with the modified enzymes. Tensile strength tests were performed on wool yarns, and it was verified that only the yarns treated with free proteases induced a significant loss of strength.

The tendency to shrink was verified by washing wool yarns three times in distilled water having 50 µL of a wetting agent for 60 minutes, at 50°C and 20 rpm, and shrinkage was quantified by the visual verification of yarn felting. It was verified that only the enzymatically treated yarns did not induce felting.

A panel of 5 experts evaluated the appearance oh the yarns and verified a better appearance of the yarns treated with proteases, compared to the control yarns.

## Claims

1. An anti-felting method of treating animal hair fibres **characterized by** the contact of the animal hair fibre with a solution of proteases that were chemically modified by glutaraldehyde and/or γ-aminopropyltriethoxysilane to increase its molecular weight in order to reduce their diffusion inside the fibre.

2. The method of claim 1 wherein the activating agent is glutaraldehyde.

3. The method of claim 1 wherein modified proteases are linked to soluble polymers.

4. The method of claim 1, wherein soluble polymers in aqueous solutions are used, like polyvinyl alcohol and/or polymers with hydroxyl groups, as support in the chemical modification of proteases.

5. A method as defined in claim 1, wherein the said proteolytic enzyme is a serine protease of bacterial origin.

6. A method, as defined in claim 5, wherein the serine protease is a *Subtilisin*.

7. The method, of claim 1, wherein the amount of protease used per Kg of wool, fibre or hair, is in the range of 1 to 1000 g.

## Patentansprüche

1. Verfahren zur Antifilzausrüstung von Tierfasem, **dadurch gekennzeichnet daß** man die Tierfasem mit einer Proteasenlösung, die durch Glutaraldehyd und/oder γ-Aminopropyltriethoxysilan chemisch modifiziert worden ist, in Berührung bringt, um das Molekular-Gewicht der Fasern zu steigern, sodaß die Diffusion derselben im Innern der Fasern vermindert wird.

2. Verfahren nach Anspruch 1 bei dem das Aktivationsmittel Glutaraldehyd ist.

3. Verfahren nach Anspruch 1 wobei die modifizierten Proteasen an lösbaren Polymer gebunden sind.

4. Verfahren nach Anspruch 1 wobei die lösbaren Polymer in wässrigen Lösungen wie z.B. Polyvinylalkohol und/oder Polymer wie z.B. Hydroxylgruppen verwendet werden, als Träger bei der chemischen Veränderung von Proteasen.

5. Verfahren nach Anspruch 1 wobei das betreffende proteolitische Enzym ein Proteasenenzym ist.

6. Verfahren nach Anspruch 5 wobei die Serinprotease Subtilisin ist.

7. Verfahren nach Anspruch 1 wobei die Menge von Protease pro Kilo Wolle, Faser oder Haar zwischen 1 bis 1000g steht.

## Revendications

1. Une méthode de traitement antifeutrant de fibres de poils d'animaux, **caractérisée par** le contact de la fibre du poil d'animal avec une solution de protéases qui ont été modifiées chimiquement par le glutaraldéhyde et/ou le γ-aminopropyltriéthoxysilane pour augmenter leur poids moléculaire afin de réduire leur diffusion à l'intérieur de la fibre.

2. La méthode de la 1^{ère} revendication où l'agent d'activation est le glutaraldéhyde.

3. La méthode de la 1^{ère} revendication où les protéases modifiées chimiquement sont liées à des polymères solubles.

4. La méthode de la 1^{ère} revendication où sont utilisés des polymères solubles dans des solutions aqueuses, tels que l'alcool de polyvinyle et/ou des polymères avec des groupes hydroxyles, comme support dans la modification chimique des protéases.

5. Une méthode selon la définition de la 1^{ère} revendication, où ladite enzyme protéolytique est une protéase à sérine d'origine bactérienne.

6. Une méthode selon la définition de la 5^{ème} revendication, où la protéase à sérine est une *Subtilisine*.

7. La méthode de la 1^{ère} revendication, où la quantité de protéases utilisée par kg de laine, de fibre ou de poil est comprise dans la plage de 1 à 1000 g.
